# EUROPEAN PATENT SPECIFICATION

(11) **EP 0 105 729 B1**
(45) Date of publication and mention of the grant of the patent: **31.05.1989**
(21) Application number: 83305890.2
(22) Date of filing: 29.09.1983
(51) Int. Cl.: D04H 1/54

(54) **Pattern densified fabric comprising conjugate fibers**
Mustermässig verdichteter, konjugierte Fasern enthaltender Stoff
Etoffe contenant des fibres conjuguées, rendue dense selon un dessin

(30) Priority: 30.09.1982 US 430307
(43) Date of publication of application: 18.04.1984
(73) Proprietor: CHICOPEE, New Brunswick New Jersey 08903 (US)
(72) Inventor: Shimalla, Charles J., Kendall Park New Jersey 08824 (US); Mays, Alfred T., East Windsor New Jersey 08520 (US)
(74) Representative: Jones, Alan John

(56) References cited:
- GB-A- 1 245 088
- GB-A- 2 078 271

## Description

Methods of compression embossing fibrous webs are known in the art. Methods of heat embossing fibrous webs including fibrous webs comprising thermoplastic fibers are also known. In general, the heat embossing is done by means of heated rollers, with the fibrous web travelling through the nip between the counterrotating heated rollers. To maintain a good through-put speed, the rollers are usually heated a few degrees higher than the melting point of the thermoplastic fibers in the web or the temperature desired in the embossing process. This is necessary so that the web travelling quickly through the nip achieves the desired temperature.

Fabrics which have been heat embossed and in particular fabrics which have been heat embossed in a pattern by patterned rollers often display damage from excessive heat. In particular, in order to achieve heat sufficient to fuse the fibers in the patterned regions, the fibers immediately adjacent the patterned regions are heated to a temperature sufficient to cause shrinkage and damage. The heat radiated to the fibers next adjacent the patterned area also shrinks the web, blurring the line of demarkation of the pattern. In the method of the present invention, a combination of heat and pressure is used to compact the fibers in the patterned regions in the web. This combination of factors does not effectively radiate to the fibers next adjacent the patterned region of the fabric, creating a fabric with very sharp pattern delineation and high loft adjacent the patterned region.

It is also old in the art to cold emboss to form or laminate fibrous layers. Cold embossing of a moist fibrous layer produces a compacted product which exhibits deformation of fibers and hydrogen bonding. Paper towelling is often made by such a method. The compaction achieved with cold embossing can be undone with water. In the method and fabric of the present invention, the compaction of the fibrous web may not be reversed or undone by the application of water.

GB-A-1 245 088 discloses a process in which a patterned fabric is produced by passing a web containing a thermoplastic through the nip of a set of rollers. One of the rollers is patterned and is heated to a temperature below the softening temperature of the thermoplastic. The pressure exerted at the nip together with the temperature of the patterned roller is sufficient to cause the thermoplastic to fuse and bond the densified regions together.

The present invention comprises a method as defined in claim 6 of pattern embossing a non-woven web of fibers comprising conjugate fibers and the fabric formed thereby. The method comprises heat embossing the web at a temperature slightly below the softening point of the low melting point component of the conjugate fiber, and with the combination of pressure and temperature sufficient to cause cold flow of at least the low melting point component of the conjugate fibers to deform and compact the conjugate fibers, compacting the fibers of the web in only the patterned regions. The fabric formed according to the method has a very sharp pattern delineation and high loft immediately adjacent the pattern. The web contains at least 15 percent conjugate fibers. In a preferred embodiment, the conjugate fibers are a sheath/core of high density polyethylene/polyester fibers. The present invention also provided a non-woven fabric as defined in claim 1.

The present invention is now described with reference to the figure which is a photomacro- graph showing a cross-section of a fabric prepared according to the method of the present invention.

The present invention comprises a method of embossing a web comprising at least 15 percent conjugate fibers and the fabric formed thereby. The conjugate fibers comprise a low melting point component and a high melting point component, and preferably comprise a sheath/core polyethylene/polyester fiber.

Preferably, the conjugate fibers employ high density polyethylene, that is, linear polyethylene that has a density of at least 0.94, and a Melt Index ("M.L") by ASTM D-1238(E) (190°C, 2160 g) of greater than 1, preferably greater than 10, and more preferably from 20 to 50. Usually the fibers will be composed of 40 to 60 weight percent, and preferably 45 to 55 weight percent, polyester, the remainder being polyethylene.

The fabrics of the invention are produced by first forming a fibrous web comprising a loose array of the conjugate fibers, as by carding or air laying. The exact weight of the fibrous web has not been found to be narrowly critical, although useful weights have been found within the range from 6.78 to 142.40 g/m² (0.2 to 4.2 ounces per square yard). This web is then conveyed to the nip of the embossing rollers.

According to the method of the present invention, a combination of heat and pressure is applied at the embossing nip combined to cause the low melting point component of the conjugate fibers of the web to cold flow. The method of the present invention encompasses using patterned embossed rolls generally known in the art. The pattern embossed rollers have raised patterned surface areas which contact and compress the web as it passes through the nip of a pair of counterrotating pattern emboss rollers. In the conventional heat embossing operation, the rollers are heated to a temperature many degrees above the effective temperature needed at the nip. This is necessary to maintain a good through-put speed of the web. The elevated temperature assures that during the short amount of time that the web spends in the nip, the effective temperature within the web is reached.

In the method of the present invention, the rollers are heated to a temperature below the softening point of the low melting point component of the conjugate fiber of the web which is to be processed through the nip of the rollers. As the web passes through the nip, the combination of heat and pressure applied by the patterned embossed rollers causes at least the low melting point component of the conjugate fibers of the web to cold flow and deform and compact the conjugate fibers, compacting the fibers in the web, in only the patterned regions. By using a combination of pressure and temperature, the method of the present invention avoids fiber shrinkage and web damage in the regions immediately adjacent the patterned regions normally caused by the radiation of heat from the superheated rollers used when heat alone is used to fuse the fibers of the web.

The fibrous webs used in practicing the method according to the present invention comprise at least 15 percent conjugate fibers and preferably sheath/core high density polyethylene/polyester conjugate fibers. Examples of other conjugate fibers which may be used in the method of the present invention are copolyester/polyester and nylon 6/nylon 66 fibers. Optionally, before passing to the nip, the web may be heated with heated air as a temperature sufficient to fuse the conjugate fibers to each other and to other fibers in the web to strengthen the fabric in the remaining, unpatterned regions.

Figure 1 illustrates a microscopic cross-section of a fabric formed according to the present invention. The fabric shown generally at 10 has embossed densified regions 12 created by the deforming and compacting of the conjugate fiber, compacting all the fibers in the web in only the pattern embossed region. The deformation and compaction of the conjugate fibers are accomplished by a combination of heat and pressure. In the method of the present invention, the heated embossed rollers are heated to a temperature slightly below the softening point of the low melting point component of the conjugate fibers. Sufficient pressure is applied in the patterned area to permanently deform the low melting point component of the conjugate fiber and hence the conjugate fiber. Any other fibers in the patterned regions of the web are compacted and the web is maintained in a densified state by the deformation of the conjugate fibers. The patterned regions display an opacity that is believed due to the air fiber interfaces. One could speculate that the deformation of the conjugate fibers is caused by cold flow of at least the sheath and perhaps the core of the fibers. In the regions 14 immediately adjacent the densified patterned regions, the fabric shows a very high loft and individual fibers 16 are seen. The high loft delineates the pattern of the fabric and indicates a lack of fiber damage in the regions immediatley adjacent the patterned regions.

## Claims

1. A non-woven fabric having high loft regions immediately adjacent densified patterned regions said fabric comprising at least 15 percent conjugate fibres having a low melting point component and another component of higher melting point, characterised in that: the densified patterned regions are unbonded and comprise compacted conjugate fibers deformed by cold flow of the low melting point component.

2. The fabric of claim 1, wherein said conjugate fibers comprises 70 to 80 percent of the fibers of said web.

3. The fabric of claim 2, wherein said conjugate fibers comprise about 75 percent of the fibers of said web.

4. The fabric of any one of claims 1 to 3, wherein the low melting point component comprises polyethylene.

5. The fabric of any one of claims 1 to 4, wherein said conjugate fibers comprise a sheath of polyethylene and a core of polyester.

6. A method of making a non-woven fabric according to any one of claims 1 to 5, comprising compressing the web in the regions to be densified under conditions of heat and pressure, characterised in that: the web is compressed at a temperature below the softening point of the low melting point component and at a combination of heat and pressure sufficient to compact and permanently deform the conjugate fibers by cold flow of the low melting point component without fuse bonding the fibers in the densified regions.

7. The method of claim 6, wherein, prior to said compression to form said densified regions, the web is heated to a temperature sufficient to fuse the conjugate fibers to each other and to other adjacent fibers in the web and thereafter cooled to a temperature below the softening point of the low melting point component.

## Patentansprüche

1. Faservliesstoff mit hochvoluminösen Bereichen unmittelbar neben verdichteten, gemusterten Bereichen, welcher Faservliesstoff wenigstens 15% Konjugatfasern enthält, die eine Komponente mit niedrigem Schmelzpunkt und eine andere Komponente mit höherem Schmelzpunkt umfassen, dadurch gekennzeichnet, daß:
die verdichteten, gemusterten Bereiche nicht gebunden sind und verdichte Konjugatfasern enthalten, die durch kalten Fluß der Komponente mit dem niedrigen Schmelzpunkt verformt worden sind.

2. Faservliesstoff nach Anspruch 1, worin die genannten Konjugatfasern 70 bis 80% der Fasern der genannten Bahn ausmachen.

3. Faservliesstoff nach Anspruch 2, worin die genannten Konjugatfasern etwa 75% der Fasern der genanten Bahn ausmachen.

4. Faservliesstoff nach einem der Ansprüche 1 bis 3, worin die Komponente mit dem niedrigen Schmelzpunkt Polyethylen umfaßt.

5. Faservliesstoff nach einem der Ansprüche 1 bis 4, worin die genannten Konjugatfasern einen Mantel aus Polyethylen und einen Kern aus Polyester umfassen.

6. Verfahren zur Herstellung eines Faservliesstoffes nach einem der Ansprüche 1 bis 5, bei welchem die Bahn in den zu verdichtenden Bereichen unter Bedingungen von Wärme und Druck komprimiert wird, dadurch gekennzeichnet, daß:
die Bahn bei einer Temperatur unterhalb des Erweichungspunktes der Komponente mit dem niedrigen Schmelzpunkt und bei einer Kombination von Wärme un Druck kompriniert wird, welche ausreicht, um die Konjugatfasern durch kalten Fluß der Koponente mit dem niedrigen Schweizpunkt zu verdichten und permanent zu verfahren, ohne die Fasern in den verdichteten Bereiche durch Schmelzen miteinander zu verbinden.

7. Verfahren nach Anspruch 6, worin die Bahn, vor dem genannten Komprimieren zur Bildung der genannten verdichteten Bereiche, auf eine Temperatur erhitzt wird, welche ausreicht, um die Konjugatfasern miteinander und mit anderen, benachbarten Fasern in der Bahn zu verschmelzen, und worin die Bahn anschliebend auf eine Temperatur unterhalb des Erweichungspunktes der Komponente mit dem niedrigen Schmelzpunkt abgekühlt wird.

## Revendications

1. Etoffe non tissée comportant des zones en relief immédiatement adjacentes aux zones profilées densifiées, ladite étoffe comprenant au moins 15% de fibres conjuguées ayant un composant à bas point de fusion et un autre composant à point de fusion plus élevé, caractérisé en ce que les zones profilées densifiées ne sont pas liées et comprennent des fibres conjuguées agglomérées qui ont été déformées par écoulement à froid du composant à bas point de fusion.

2. Etoffe selon la revendication 1, dans laquelle lesdites fibres conjuguées représentent de 70 à 80% des fibres dans ladite bande.

3. Etoffe selon la revendication 2, dans laquelle lesdites fibres conjuguées constituent environ 75% des fibres de ladite bande.

4. Etoffe selon l'une quelconque des revendications 1 à 3, dans laquelle le composant à bas point de fusion comprend du polyéthylène.

5. Etoffe selon l'une quelconque des revendications 1 à 4, dans laquelle lesdites fibres conjuguées comprennent une gaine en polyéthylène et une âme en polyester.

6. Procédé de fabrication d'une étoffe non tissée selon l'une quelconque des revendications 1 à 5, consistant à comprimer la bande dans les zones à densifier dans des conditions de chaleur et de pression, caractérisé en ce qu'on comprime la bande à une température inférieure au point de ramollissement du composant à bas point de fusion et à l'aide d'une combinaison de chaleur et de pression suffisante pour agglomérer et déformer de façon permanente les fibres conjuguées par écoulement à à froid du composant à bas point de fusion, sans lier par fusion les fibres dans la région densifiée.

7. Procédé selon la revendication 6, dans lequel, avant ladite compression pour former lesdites régions densifiées, on chauffe la bande à une température suffisante pour fusionner ensemble les fibres conjuguées ainsi que d'autres fibres adjacentes et qu'ensuite on refroidit à une température inférieure au point de ramollissement du composant à bas point de fusion.
